

## UNITED STATES PATENT OFFICE

2,212,603

## COATING COMPOSITION

Cleveland B. Hollabaugh, Wilmington, Del., assignor to Hercules Powder Company, Wilmington, Del., a corporation of Delaware

No Drawing. Application September 16, 1937,  
Serial No. 164,237

20 Claims. (Cl. 134—79)

This invention relates to coating compositions and to articles coated therewith. More particularly it relates to coating compositions suitable for the production of highly flexible films which are tack-free, even at slightly elevated temperatures and to a flexible base coated with such compositions.

Nitrocellulose, cellulose acetate, cellulose acetobutyrate, cellulose aceto-propionate, chlorinated rubber, synthetic resins and similar film-forming materials, when used alone, produce films which are brittle and unsuited for coating a very flexible base. To produce flexible films by the use of such film-forming materials, it is necessary to add a softening or plasticizing agent to the film-forming material. However, the addition of plasticizing or softening agents to film-forming materials have a tendency to render them tacky, particularly at slightly elevated temperatures.

In the formulation of protective and decorative coatings for application to a very flexible base, such as paper, cloth, metallic foil, and the like, it is very difficult to produce a film which is highly flexible over the ordinary range of temperatures at which the coated materials is used and yet not sufficiently tacky to have a tendency to cling together at normal temperatures and to adhere firmly together when in contact under pressure as when stored in piles for long periods, particularly at the slightly elevated temperatures which may be encountered on storage in the summer in warehouses and freight cars.

The tendency of the coated surfaces to cling together and have excessive resistance to slip, or "cling" as it is termed in the art, is highly objectionable. The tendency to adhere firmly together may and frequently does cause practically a total loss of the coated product and, hence, is even more serious.

Thus, it is often found that sheets of paper coated with a flexible lacquer piled in stacks and allowed to stand for a long period of time, or at slightly elevated temperatures, or both, will adhere firmly together to form a solid mass, even though the lacquer coating was entirely dry before the sheets were stacked and even though the coating was not soft or tacky to the touch. This phenomena is termed "blocking" by the art. Blocking is exaggerated by pressure and it will be found that the lower sheets of a stack which are under more weight than the upper sheets will block more readily than the upper sheets. There is no known way of separating sheets which have been blocked without damaging them, so blocking will cause practically a total loss of the blocked material.

It will be appreciated that blocking is not limited to coated sheets of paper but can occur when any two coated surfaces or when a coated

surface and an uncoated surface are in close contact. Thus, a roll of coated paper, cloth, or metal foil which is tightly wound can readily block into a solid mass which cannot be unwound.

In order to avoid blocking of lacquered surfaces, it has been the practice heretofore to coat upon a surface only very small amounts of lacquer solids, so that the surface was incompletely covered. The exposed areas of the base surface, 10 protruding fibers in the case of paper and cloth bases, and lacquer film irregularities are sufficient to temporarily prevent blocking. Such coatings are, however, inferior in their appearance and in their resistance to water-vapor, 15 water, grease and the like, and will eventually block.

Another serious difficulty is frequently encountered when coating both sides of a flexible base, such as paper and the like. In coating paper on both sides, one side of the paper is ordinarily coated, the coating dried at an elevated temperature, and then the opposite side coated by a second pass through the coating machine. Usually the side which is last coated and dried will have 25 faulty spots resembling bubbles or craters. These faulty spots are apparently caused by residual solvent absorbed on the paper fibers from the lacquer applied on the first side coated evaporating through the second coating before it 30 is entirely dry. By the time the solvent vapors have broken through the coating on the second side coated, it is usually so viscous that it does not flow and close up the holes left by the broken bubbles.

The object of this invention is to provide a coating composition which will dry to a film which is flexible over the range of ordinary atmospheric temperatures and yet which is free of cling and which shows little or no tendency 40 to block even when stored at slightly elevated temperatures. This object is accomplished by the addition of a relatively small quantity of an alkali metal salt of a higher aliphatic sulfate to a flexible coating composition. Such an addition will eliminate the tendency of the flexible coating composition, when in the form of a film on a flexible surface, to cause blocking, with the consequent losses attendant thereto. Such an addition has a further effect and one which is 45 likewise quite valuable. I have found that coating compositions in accordance with this invention, when used to coat both sides of paper, are ordinarily entirely free of any tendency to show faults in the coating applied to the second side 50 coated.

While my primary objective is to provide a coating composition suitable for application to a flexible base, it will be appreciated that my coating composition is by no means limited to such 55

uses, but will be found useful for application to any typical surface on which a slick surface, free of a tendency to cling, is desired. In this connection it will be appreciated that coating compositions which are of the hard, glossy type frequently show a tendency to cling, particularly when at slightly elevated temperatures. It will be found that the addition of an alkali metal salt of a higher aliphatic sulfate to such coating compositions, for example, furniture lacquers and the like, will cause the final film to be free of cling and present a very slick surface which is less readily scuffed and marred than surfaces which have a slight cling.

15 A further object of this invention is to provide a flexible sheet material coated with a uniform protective and decorative coating which is substantially free of cling and which is not subject to blocking. This object is accomplished by 20 coating a flexible base material with the coating composition in accordance with this invention.

The coating composition in accordance with this invention will comprise essentially a film-forming material, such as, for example, a cellulose ester, as nitrocellulose, cellulose acetate, cellulose propionate, cellulose butyrate, cellulose aceto-propionate, cellulose aceto-butyrate, etc., chlorinated rubber, synthetic resins, and the like; and an alkali metal salt of a higher aliphatic sulphate. The alkali metal salt of the higher aliphatic sulphate which I include in this composition has the property of giving the coating a tack-free surface, even though a plasticizing or softening agent is presented in amounts which would 35 give a tacky surface in its absence.

The alkali metal salt of the higher aliphatic sulphate which I may use will contain eight or more carbon atoms and may be, for example, sodium oleyl sulphate, sodium lauryl sulphate, sodium 40 stearyl sulphate, sodium myristyl sulphate, sodium cetyl sulphate, etc., or mixtures thereof. The amount of the alkali metal salt of a higher aliphatic sulfate which I include in my composition will depend upon the various other formulating ingredients included therein. It will be 45 present in amount sufficient to have the desired anti-cling and anti-blocking action, but ordinarily in amount insufficient to give the film a flat appearance, and always in amount insufficient to give the film a frosted appearance.

50 While the amounts of the alkali metal salt of the higher aliphatic sulphate which may be used in the coating compositions in accordance with this invention will vary somewhat with the nature and the amounts of the other ingredients present, I have found that an amount within the range of about 0.50% to about 1.25% of the material in the composition which remains in the final film will be found satisfactory. Immediate effects do not ordinarily appear using concentrations between 0.50% and 0.70% until the film produced by drying the composition has aged about a week. Amounts of the alkali metal salt of the higher aliphatic sulfate above about 1.5% 60 by weight of the film-forming solids in the composition ordinarily causes a noticeable reduction in the gloss or a "flattening" of the film.

The film-forming material used in the composition in accordance with this invention may 70 be, for example, a cellulose ester, such as, nitrocellulose, cellulose acetate, cellulose aceto-butyrate, cellulose aceto-propionate, cellulose butyrate, cellulose propionate; chlorinated rubber; synthetic resins, as, polybasic acid-polyhydric alcohol resins, etc. The nitrocellulose used may

be any of the types used in coating compositions, as, for example, a nitrocellulose having a nitrogen content within the range of about 10.9% to about 12.3%. Similarly, the other cellulose esters which may be used will be of the usual protective 5 coating types. Thus, the cellulose acetate may have an acetyl content expressed as acetic acid, within the range of about 50% to about 62.5% by weight, and preferably within the range of about 52% to about 56.5%. The cellulose aceto-butyrate may vary in composition over the entire possible range from straight cellulose acetate to straight cellulose butyrate, and may be either of the hydrolyzed or unhydrolyzed types. Preferably the cellulose acetobutyrate will have an 15 acetyl-butyryl content within the range of about 45% acetyl-12% butyryl to about 35% acetyl-22% butyryl, by weight. The cellulose acetopropionate may vary in composition from straight cellulose acetate to straight cellulose propionate, 20 but will preferably have an acetyl-propionyl content within the range of about 15% acetyl-35% propionyl to about 25% acetyl-45% propionyl by weight. Likewise, the chlorinated rubber may be of any of the usual protective coating types, 25 and may have a chlorine content within the range of about 50% to about 73% by weight, and preferably within the range of about 60% to about 69% by weight.

The film-forming material which I may use 30 may have a viscosity characteristic of within a comparatively wide range depending upon the characteristics desired of the composition. When it is desirable to utilize the film-forming material in the form of a solution having a high 35 viscosity therewith in depositing a thin film, a high viscosity characteristic film-forming material will be utilized. On the other hand, when it is desired to deposit a relatively heavy film, by the use of a low viscosity solution, a low film-forming material having a low viscosity characteristic will be used. Thus, when using a nitrocellulose as a film-forming ingredient it will have a viscosity characteristic within the range of about .0125 second (Hercules) to about 400 seconds (Hercules). The nitrocellulose which I ordinarily employ will have a viscosity characteristic within the narrower range of about 0.1 second (Hercules) to about 100 seconds (Hercules). The other film-forming ingredients which I may 45 use will have viscosity characteristics within corresponding ranges.

In addition to the alkali metal salt of a higher aliphatic sulfate and a film-forming ingredient, the coating compositions in accordance with this 55 invention may contain other formulating ingredients, such as, softeners or plasticizers, natural resins, synthetic resins, pigments, dyes, etc. The plasticizing or softening agent which I may use in the coating compositions in accordance with 60 this invention may be present in widely varying amounts depending upon the characteristics desired in the ultimate film, the character of the film-forming material utilized, and the exact characteristic of the plasticizing or softening 65 agent employed. With film-forming ingredients such as, nitrocellulose, cellulose acetate, chlorinated rubber, etc., and normally effective plasticizers such as diethyl or dibutyl phthalate, etc., the plasticizer will ordinarily be present in amount 70 within the range of about 20% to about 40% by weight of the film-forming material present in the composition, and desirably within the range of about 25% to about 35%. It will be appreciated, however, that when using certain types of 75

film-forming ingredients, such as, highly flexible synthetic resins, no plasticizer or softener is necessary even in compositions intended for application to highly flexible surfaces.

- 5 The plasticizing or softening agent which I may use may be for example, dibutyl phthalate, diethyl phthalate, tricresyl phosphate, triethyl citrate, methyl phthalyl methyl glycolate, methyl phthalyl butyl glycolate, tributyl phosphate, cas-  
 10 tor oil, substituted castor oils, and the like. The composition may, in addition, contain gums, resins, pigments, and other formulating ingredients ordinarily used in protective coating compositions of this type. The gum or resins employed  
 15 may be, for example, dammar gum, ester gum, methyl abietate, modified alkyd resins, terpinene maleate resins and the like.

The composition in accordance with this invention may be applied to a flexible base in the form of a solution dissolved in suitable organic solvents known to the art. The particular organic solvent utilized may be a single organic compound, but will ordinarily be an admixture of various solvents and non-solvents, of different rates of composition. The particular solvents chosen will depend primarily on the film-forming material included in the composition.

When applied in the form of a solution it will be found that the alkali metal aliphatic sulphate contained in the composition will be dissolved in the organic solvent or will be partially dissolved and partially dispersed as a very fine suspension. In either case, it will be deposited uniformly in the ultimate film produced on evaporating the solvent.

The viscosity of the solution to be utilized will ordinarily be chosen with reference to the method by which it is to be applied to the flexible base, and may be conveniently controlled by the concentration of the film-forming ingredient in the solution or by the viscosity characteristic of the particular lot of the film-forming ingredient utilized. Thus, for application by spraying, the solution will desirably not exceed a viscosity of about 100 centipoises. For application by roller coating, a higher viscosity may be used, such as, for example, a viscosity within the range of about 100 centipoises to about 800 centipoises, and preferably within the range of about 500 centipoises to about 750 centipoises. For application by means of a doctor blade still higher viscosities may be employed.

Compositions in accordance with this invention, suitable for application in the form of solutions are more specifically illustrated by the examples given in Table I.

TABLE I

|    |                                               | Example No. |      |      |      |
|----|-----------------------------------------------|-------------|------|------|------|
|    |                                               | 1           | 2    | 3    | 4    |
| 65 | Nitrocellulose (Hercules-R. S. 1/2 Sec. type) | 50.0        | 69.2 | 69.2 | 55.0 |
|    | Terpene-maleic anhydride synthetic resin      | 25.0        |      |      |      |
|    | Oil-modified alkyd resin                      |             |      | 44.0 |      |
| 70 | Dibutyl phthalate                             | 24.1        | 30.0 |      |      |
|    | Butyl phthalyl butyl glycolate                |             |      | 30.0 |      |
|    | Sodium lauryl sulfate                         | 0.9         | 0.8  | 0.8  | 1.0  |

A suitable solvent mixture for the compositions listed in Table I is as follows:

|               | Per cent |
|---------------|----------|
| Butyl acetate | 20       |
| Ethyl acetate | 25       |
| Butanol       | 5        |
| Toluol        | 50 5     |

The amount of the solvent utilized will depend upon the method by which the compositions are to be applied.

Compositions in accordance with this invention, suitable for application in the form of a solution are further illustrated by the following examples. In each of these examples, the amount of solvent used will depend upon the viscosity desired for the particular method of application to be used.

#### Example 5

|                       | Parts by weight |
|-----------------------|-----------------|
| Cellulose acetate     | 25.0            |
| Dibutyl phthalate     | 15.7 20         |
| Sodium lauryl sulfate | 0.3             |
| Solvent mixture:      |                 |
| Methyl-ethyl ketone   | 2               |
| Diacetone alcohol     | 1               |
| Acetone               | 1 25            |

#### Example 6

|                                                          | Per cent |
|----------------------------------------------------------|----------|
| Chlorinated rubber                                       | 70.6     |
| Butyl phthalyl butyl glycolate                           | 28.5 30  |
| Sodium lauryl sulfate                                    | 0.9      |
| Solvent mixture:                                         |          |
| Hydrogenated petroleum hydrocarbon solvent (solvesso #2) | parts 2  |
| Toluol                                                   | do 1 35  |

#### Example 7

|                                 | Per cent |
|---------------------------------|----------|
| Cellulose aceto-butyrate        | 55.2     |
| Methyl phthalyl ethyl glycolate | 44.1     |
| Sodium lauryl sulfate           | 0.7 40   |
| Solvent mixture:                |          |
| Diacetone alcohol               | parts 1  |
| Methyl ethyl ketone             | do 3     |
| Acetone                         | do 4     |

#### Example 8

|                                                       | Per cent |
|-------------------------------------------------------|----------|
| Ethylene glycol ester of terpinene maleic anhydride   | 83.7     |
| Diethylene glycol ester of terpinene maleic anhydride | 15.0 50  |
| Sodium lauryl sulfate                                 | 1.25     |

This composition may be applied in the form of a solution in a suitable solvent, such as, toluol.

#### Example 9

|                                                     | Parts |
|-----------------------------------------------------|-------|
| Ethylene glycol ester of terpinene maleic anhydride | 82    |
| Stearic triglyceride (hydrogenated castor oil)      | 18 60 |
| Ethyl cellulose (low viscosity type)                | 3     |
| Sodium lauryl sulfate                               | 1.3   |

This composition may be applied in the form of a solution in a suitable solvent, such as, a mixture of 20% butanol and 80% toluol.

Alternately, the composition in accordance with this invention may be applied to a base in the form of a substantially water-immiscible solution emulsified in disperse phase in water. When applied in the form of an emulsion, the alkali metal higher aliphatic sulphate may be dissolved in the lacquer solution, or in the aqueous phase, or in both, and will function as emulsifying agent for dispersing the water-immiscible

solution, as well as for a tack-reducing agent in the ultimate film. The alkali metal higher aliphatic sulphate may be the sole emulsifying agent used or it may be used in conjunction with other emulsifying agents. When dissolved or suspended in only the protective coating solution, I have found that it is less efficient in its emulsifying action, than when dissolved in the aqueous phase of the emulsion, and that it is desirable to utilize another emulsifying agent in the aqueous phase to secure efficient emulsification of the composition.

In utilizing the coating composition in accordance with this invention in the form of an emulsion in water, it will be found that the viscosity of the emulsion can be conveniently controlled to adapt the emulsion for application by various methods, and it will be found that the emulsion may be applied by any of the usual methods for application of ordinary protective coating solutions. On the other hand, the viscosity of the water-immiscible solution of the protective coating composition which is dispersed may be utilized to control its penetration into the pores of the base to which it is applied, and provides a very convenient and flexible method for such control, particularly when applying the compositions to a highly porous flexible base.

I have found that, even though the particle sizes of the disperse phase of the emulsion be less than the pore sizes of the porous material, and even though the viscosity of the emulsion be very low, so that one would expect rapid penetration of the porous support by the emulsion, substantially no penetration occurs provided the dispersed protective coating solution be of sufficiently high viscosity as compared with ordinary protective coating solutions adapted, for example, for application by spraying. In other words, the viscosity and not the particle size of the disperse phase of the emulsion is the determining factor of penetration of the porous support by the emulsion.

To obtain the best results in the application of my emulsions to porous surfaces, it is desirable to correlate the porosity of absorbency of the porous support with the viscosity of the disperse phase of the emulsion, for example, with a high porous support such as a high absorbent paper, I prefer to use an emulsion which, while fluid and free-running as an emulsion contains as the disperse phase a protective coating solution of relatively high viscosity, to the end that, after most of the aqueous phase of the emulsion has been absorbed by the porous support, or evaporated, or otherwise removed, the disperse phase coalesces and deposits as a highly viscous coating on the very surface of the support and does not penetrate thereinto, and such disperse phase only then solidifies by the elimination of the solvents in such dispersed phase.

When applying the protective coating composition in accordance with this invention in emulsified form to a highly porous surface which absorbs a relatively high percentage of the aqueous phase, and when utilizing the alkali metal aliphatic sulfate as the emulsifying agent, it is desirable either to increase the amount of the alkali metal aliphatic sulphate dissolved in the aqueous phase, or to add it both to the aqueous phase and to the dispersed phase, so that the ultimate film produced by the drying of the composition will contain an amount of the alkali metal aliphatic sulphate as hereinbefore specified. It will be appreciated that when a portion of the aqueous phase

of the emulsion is absorbed into the bodies of the flexible material which is coated, the amount of the alkali metal aliphatic sulphate deposited in the ultimate film is proportionately decreased.

I have been unable to determine any numerical relation between pore size of the porous support and the viscosity in the disperse phase of the protective coating emulsion. However, the following examples of emulsified compositions in accordance with this invention in which nitrocellulose is utilized as the film-forming ingredient, and which are adapted for application to surfaces of different porosity, will enable those skilled in the art, with ease, to economically and efficiently apply the coating compositions to any porous, absorbent base desired to be coated. It will be appreciated that in each of these compositions, the alkali metal salt of the higher aliphatic sulfate may be dissolved either in the lacquer phase or the aqueous phase of the emulsion, or both, as may be desired.

Thus, by way of example, with a highly porous, absorbent surface of blotting paper, it has been found that, with an emulsion containing in the disperse phase a nitrocellulose solution of a viscosity of 10,000 seconds (A. S. T. M.), a continuous, non-porous, adherent, substantially non-penetrating coating of nitrocellulose can be formed on the surface when as little as 14 lbs. per 3000 square feet of dry substance is deposited.

Similarly, with a jute cardboard, it has been found that with an emulsion containing the disperse phase a nitrocellulose solution of a viscosity of 1000 seconds (A. S. T. M.) a continuous, non-porous, adherent, substantially non-penetrating coating of nitrocellulose can be formed on the surface when as little as 11 lbs. per 3000 square feet of dry substance is deposited.

Similarly, with Lion jute tag cardboard, a substantially less porous cardboard, it has been found that with a disperse nitrocellulose phase of a viscosity of 150 seconds (A. S. T. M.) a continuous, non-porous, adherent, substantially non-penetrating coating of nitrocellulose can be formed on the surface thereof with as little as 7 lbs. per 3000 square feet of dry substance deposited.

Similarly, with Champion Garamond Text paper, a relatively porous paper, it has been found that with a nitrocellulose emulsion containing in the disperse phase a nitrocellulose solution of a viscosity of 250 seconds (A. S. T. M.), a continuous, non-porous, adherent, non-penetrating coating of nitrocellulose can be formed on the surface when as little as 10 lbs. per 3000 square feet of dry substance is deposited.

Similarly, with plain bond paper, with an emulsion having a disperse phase of 20 second (A. S. T. M.), viscosity nitrocellulose solution, a continuous, non-porous, adherent substantially non-penetrating coating of nitrocellulose can be formed on the surface with 7 lbs. of dry substance per 3000 square feet of surface.

Similarly, with Fernside Ledger paper, a less porous paper, with an emulsion having a disperse phase of a nitrocellulose solution of a viscosity of 10 seconds (A. S. T. M.), a continuous, non-porous adherent, substantially non-penetrating coating of nitrocellulose can be formed on the surface with as little as 5 lbs. per 3000 square feet of dry substance.

In using the composition in accordance with this invention in the form of an emulsion, it will be dissolved in a substantially water-immiscible solvent mixture, admixed with an aqueous solu-

- tion of an alkali metal higher aliphatic sulfate or other emulsifying agent, and passed through a suitable colloid mill or homogenizer. If desired the alkali metal salt of the higher aliphatic sulfate may be omitted entirely from the water-immiscible solution of the film-forming material, and included only in the aqueous phase of the emulsion in which it will function as the emulsifying agent. Alternately it may be included only in the lacquer phase of the emulsion and another emulsifying agent added to the aqueous phase, or it may be included in both phases. When it is desired to use another emulsifying agent in the aqueous phase it will be found the emulsifying agent utilized may be for example, a sulphonated oil, as sulphonated castor oil, etc. a soap, as, sodium oleate, sodium stearate, the corresponding potassium salts, etc., a sodium salt of butyl or isopropyl naphthalene sulphonic acid, as sodium butyl naphthalene sulphonate, etc., oleo glycerol sulphate, methyl cellulose, the sodium salt of sulphuric ester of glycerin-mono-dodecyl ether, the sodium salt of dodecyl-mercapto acetic acid, etc., or other compounds equivalent therefor, or mixtures thereof.

The emulsifying agent may be used in widely varying amount, depending upon the particular emulsifying agent used, thus, for example, in amount within about the range 0.1%--5% by weight of the water. By way of example, 2% of sodium resinate or 0.75% of sodium lauryl sulphate in the water phase will be satisfactory.

In preparing an emulsified composition in accordance with this invention the substantially water-immiscible solution of the film-forming material utilized will be emulsified in disperse phase in aqueous solution of the emulsifying agent on a ratio within the range of about 1.75:1 to about 4:1 and preferably on a ratio within the range of about 2:1 to about 3:1. From the standpoint of economy, it is desirable that the solution of the film-forming material so emulsified be of sufficiently high viscosity that it will not penetrate into the surface of the flexible base to be coated to any substantial amount. The viscosity of the solution of the film-forming material will ordinarily fall within the range of about 3 seconds to about 27,000 seconds and more desirably within the range of about 150 seconds to about 10,000 seconds, as determined by the A. S. T. M. standard method, that is the time required for a  $\frac{1}{8}$ " ball to fall through 10 inches of the solution contained in a 1" diameter tube at 25° C.

The solvent mixture employed in the substantially water-immiscible solution of nitrocellulose may have an average boiling point within a rather wide range, and it will be found in general that the more porous the surface to be coated the more the average boiling range of the solvent mixture can be. It is believed that the reason for this is the fact that a porous surface absorbs the aqueous phase of the emulsion so that it does not interfere with the evaporation of the solvent in the disperse phase and that absorption of the aqueous phase is dependent upon the porosity of the surface. When using nitrocellulose as the film-forming ingredient in emulsified compositions in accordance with this invention which are intended to be applied to flexible surfaces, which are relatively high porosity, it will be found that more than half of the solvent or solvent mixtures will boil below a 140° C. or within the range of about 150° C.-130° C. In the formulation of the solvent mixture there will be found that the sol-

vents and diluents listed in the following table and within the maximum amounts given may be used.

| No. | Approximate boiling point, °C. | Name                                      | Maximum percent to be used in solvent mixture | 5  |
|-----|--------------------------------|-------------------------------------------|-----------------------------------------------|----|
| 1   | 35                             | Ether                                     | 10                                            |    |
| 2   | 56                             | Acetone                                   | 25                                            |    |
| 3   | 50+                            | Mineral spirits                           | 75                                            |    |
| 4   | 60                             | Methyl acetate                            | 50                                            |    |
| 5   | 63                             | Methanol                                  | 25                                            |    |
| 6   | 75                             | Ethyl acetate                             | 100                                           |    |
| 7   | 76                             | Carbon tetrachloride                      | 50                                            |    |
| 8   | 78                             | Ethanol                                   | 25                                            | 15 |
| 9   | 80                             | Benzol                                    | 100                                           |    |
| 10  | 80                             | Ethyl methyl ketone ethyl acetone         | 25                                            |    |
| 11  | 80                             | Isopropyl alcohol                         | 75                                            |    |
| 12  | 85                             | Ethylene chloride                         | 75                                            |    |
| 13  | 90                             | Isopropyl acetate                         | 100                                           |    |
| 14  | 98                             | Ethyl propionate                          | 100                                           |    |
| 15  | 100                            | Diethyl carbonate                         | 100                                           | 20 |
| 16  | 101                            | Diethylene oxide                          | 100                                           |    |
| 17  | 102                            | Butanol                                   | 75                                            |    |
| 18  | 110                            | Toluol                                    | 100                                           |    |
| 19  | 113                            | Butyl acetate                             | 100                                           |    |
| 20  | 115                            | Amyl alcohol                              | 75                                            |    |
| 21  | 118                            | Methyl isobutyl ketone                    | 100                                           |    |
| 22  | 120                            | Methyl cellosolve                         | 25                                            | 25 |
| 23  | 125                            | Epiethylin glycidylethyl ether            | 100                                           |    |
| 24  | 126                            | Pentasol                                  | 100                                           |    |
| 25  | 130                            | Isoamyl alcohol isobutyl carbinol primary | 25                                            |    |
| 26  | 130                            | Cellosolve                                | 25                                            |    |
| 27  | 135                            | Ethyl benzene                             | 75                                            |    |
| 28  | 135                            | Butyl ethyl carbonate                     | 100                                           |    |
| 29  | 135                            | Pent-acetate                              | 100                                           | 30 |
| 30  | 139                            | Xylool                                    | 75                                            |    |
| 31  | 139                            | Butyl propionate                          | 100                                           |    |

As illustrative of emulsified compositions, made in accordance with this invention and suitable for application to porous surfaces, Examples 10-15, inclusive, may be cited. In each of these examples the formulae of lacquer phase is given, and it will be understood that each of these solutions is emulsified in disperse phase in water containing 0.75% by weight of sodium lauryl sulfate on a ratio of 3 parts of the solution to 1 part of water.

#### Example 10

|                                        | Parts | 45 |
|----------------------------------------|-------|----|
| Nitrocellulose (any desired viscosity) | 25    |    |
| Castor oil                             | 38    |    |
| Sodium lauryl sulfate                  | 0.5   |    |
| Ethyl alcohol                          | 10    | 50 |
| Butyl acetate                          | 14    |    |
| Toluol                                 | 14    |    |

Using  $\frac{1}{2}$  second (Hercules) nitrocellulose—solution viscosity (steel ball supra) is 500 seconds. 55

#### Example 11

|                         | Parts |    |
|-------------------------|-------|----|
| Nitrocellulose          | 20    |    |
| Castor oil              | 30    | 60 |
| Sodium myristyl sulfate | 0.3   |    |
| Ethyl alcohol           | 9     |    |
| Butyl acetate           | 21    |    |
| Toluol                  | 20    | 65 |

Using  $\frac{1}{2}$  second (Hercules) nitrocellulose—solution viscosity (steel ball, supra) is 60 seconds.

Using 1 second (Hercules) nitrocellulose—solution viscosity (steel ball, supra) is 250 seconds. 70

Using 5 second (Hercules) nitrocellulose—solution viscosity (steel ball, supra) is 3000 seconds.

Using 18 second (Hercules) nitrocellulose—solution viscosity (steel ball, supra) is 10,000 seconds. 75

## Example 12

|                                                                                                               | Parts |
|---------------------------------------------------------------------------------------------------------------|-------|
| Nitrocellulose                                                                                                | 10    |
| Castor oil                                                                                                    | 15    |
| 5 Sodium lauryl sulfate                                                                                       | 0.18  |
| Ethyl alcohol                                                                                                 | 4     |
| Butyl acetate                                                                                                 | 36    |
| Toluol                                                                                                        | 35    |
| 10. Using $\frac{1}{2}$ second (Hercules) nitrocellulose—solution viscosity (steel ball, supra) is 2 seconds. |       |
| Using 5 second (Hercules) nitrocellulose—solution viscosity (steel ball, supra) is 20 seconds.                |       |
| Using 18 second (Hercules) nitrocellulose—solution viscosity (steel ball, supra) is 100 seconds.              |       |
| 15. Using 110 second (Hercules) nitrocellulose—solution viscosity (steel ball, supra) is 250 seconds.         |       |
| Using 200 second (Hercules) nitrocellulose—solution viscosity (steel ball, supra) is 1000 seconds.            |       |
| 20. Using 400 second (Hercules) nitrocellulose—solution viscosity (steel ball, supra) is 10,000 seconds.      |       |

## Example 13

|                                                        | Parts |
|--------------------------------------------------------|-------|
| 25. 1000 second (Hercules) nitrocellulose              | 5     |
| Castor oil                                             | 7     |
| Sodium lauryl sulfate                                  | 0.08  |
| Butyl acetate                                          | 43    |
| Toluol                                                 | 43    |
| 30. Solution viscosity (steel ball, supra)—30 seconds. |       |

## Example 14

|                                                          | Parts |
|----------------------------------------------------------|-------|
| 35. $\frac{1}{2}$ second (Hercules) nitrocellulose       | 38.5  |
| Triethyl citrate                                         | 23    |
| Sodium lauryl sulfate                                    | 0.4   |
| Butyl acetate                                            | 11    |
| Ethyl alcohol                                            | 16.5  |
| Toluol                                                   | 11    |
| 40. Solution viscosity (steel ball, supra)—1800 seconds. |       |

## Example 15

|                                                         | Parts |
|---------------------------------------------------------|-------|
| 45. $\frac{1}{2}$ second (Hercules) nitrocellulose      | 35    |
| Triethyl citrate                                        | 21    |
| Sodium lauryl sulfate                                   | 0.4   |
| Alcohol                                                 | 14    |
| Butyl acetate                                           | 16    |
| Toluol                                                  | 16    |
| 50. Solution viscosity (steel ball, supra)—310 seconds. |       |

It will be understood that a wide variety of solvent mixtures may be used in place of those given in the above formulae, so long as the solvent and diluents be chosen so that more than half of the solvent mixture boils below about 140° C.

It will now be observed that the emulsions in accordance with this invention are characterized by the inclusion of a viscous nitrocellulose solution including a solvent or solvent mixture more than half of which is low boiling, i. e. below 140° C. and having a high solids or non-volatile content, and the solution being within a particular range of ratio with respect to the water phase of the emulsion.

In use for the coating of porous materials, the emulsion in accordance with this invention and having a nitrocellulose solution phase of suitable or desired viscosity with respect to the porosity of the material to be coated, will be applied in any desired manner. On application of the emulsion, it will break, either from physical action, as the absorbence of the water phase by the absorbent material, or from the solution in the

water phase of an electrolyte carried by the material, or both with resultant coalescence of the disperse phase on the surface of the material with the formation of a continuous, non-porous film on the surface, on evaporation of the solvent. 5 Due to the fact that the water of the emulsion is absorbed by the porous material, the water does not have to be evaporated with the solvent, and consequently, despite the low boiling point of the solvent or solvent mixture and the higher concentration of solids, the coalesced solution will dry to a clear film where no pigment is present and in any event to a film free from precipitated nitrocellulose.

This application is a continuation-in-part of 15 my application for United States patent, Serial No. 123,725, filed February 2, 1937, (now United States Patent No 2,101,066), which is in turn a continuation in part of applications Serial No. 11,685, filed March 18, 1935, and Serial No. 12,725, 20 filed March 23, 1935, which are continuations-in-part of application filed by me Serial No. 703,833, filed December 23, 1933 (now United States Patent No. 2,044,571).

What I claim and desire to protect by Letters 25 Patent is:

1. In a film-forming protective and decorative lacquer composition of the type in which a film-forming material is dissolved in a non-aqueous, 30 volatile, organic solvent, or solvent mixture, and in which the film-forming material comprises a material selected from the group consisting of cellulose esters, chlorinated rubber, synthetic resins and mixtures thereof, the improvement 35 which consists in adding to the lacquer composition an alkali metal aliphatic sulphate which contains at least eight carbon atoms, said sulphate being present in the said composition in an amount insufficient to cause substantial flattening of the gloss of the film produced by the use 40 of the said lacquer composition but sufficient to insure deposition with and incorporation in the film in an amount between about 0.5% and about 1.25%, by weight, of the deposited film, the said film produced by the use of the said lacquer composition being characterized by possessing high 45 gloss and by being substantially non-tacky and non-blocking.

2. In a film-forming protective and decorative lacquer composition of the type in which a film-forming material is dissolved in a non-aqueous, volatile, organic solvent, or solvent mixture, and in which the film-forming material comprises a cellulose ester, the improvement which consists in adding to the lacquer composition an alkali 55 metal aliphatic sulphate which contains at least eight carbon atoms, said sulphate being present in the said composition in an amount insufficient to cause substantial flattening of the gloss of the film produced by the use of the said lacquer 60 composition but sufficient to insure deposition with and incorporation in the film in an amount between about 0.5% and about 1.25%, by weight, of the deposited film, the said film produced by the use of the said lacquer composition being 65 characterized by possessing high gloss and by being substantially non-tacky and non-blocking.

3. In a film-forming protective and decorative lacquer composition of the type in which a film-forming material is dissolved in a non-aqueous, 70 volatile, organic solvent, or solvent mixture, and in which the film-forming material comprises a chlorinated rubber, the improvement which consists in adding to the lacquer composition an alkali metal aliphatic sulphate which contains at 75

least eight carbon atoms, said sulphate being present in the said composition in an amount insufficient to cause substantial flattening of the gloss of the film produced by the use of the said lacquer composition but sufficient to insure deposition with and incorporation in the film in an amount between about 0.5% and about 1.25%, by weight, of the deposited film, the said film produced by the use of the said lacquer composition being characterized by possessing high gloss and by being substantially non-tacky and non-blocking.

4. In a film-forming protective and decorative lacquer composition of the type in which a film-forming material is dissolved in a non-aqueous, volatile, organic solvent, or solvent mixture, and in which the film-forming material comprises a synthetic resin, the improvement which consists in adding to the lacquer composition an alkali metal aliphatic sulphate which contains at least eight carbon atoms, said sulphate being present in the said composition in an amount insufficient to cause substantial flattening of the gloss of the film produced by the use of the said lacquer composition but sufficient to insure deposition with and incorporation in the film in an amount between about 0.5% and about 1.25%, by weight, of the deposited film, the said film produced by the use of the said lacquer composition being characterized by possessing high gloss and by being substantially non-tacky and non-blocking.

5. In a film-forming protective and decorative lacquer composition of the type in which a film-forming material is dissolved in a non-aqueous, volatile, organic solvent, or solvent mixture, and in which the film-forming material comprises nitrocellulose, the improvement which consists in adding to the lacquer composition an alkali metal aliphatic sulphate which contains at least eight carbon atoms, said sulphate being present in the said composition in an amount insufficient to cause substantial flattening of the gloss of the film produced by the use of the said lacquer composition but sufficient to insure deposition with and incorporation in the film in an amount between about 0.5% and about 1.25%, by weight, of the deposited film, the said film produced by the use of the said lacquer composition being characterized by possessing high gloss and by being substantially non-tacky and non-blocking.

6. An article comprising a base at least one of the surfaces of which is coated with a protective and decorative, glossy, substantially non-blocking and non-tacky, film, produced by the evaporation of the solvent from the lacquer composition defined in claim 1.

7. An article comprising a base at least one of

the surfaces of which is coated with a protective and decorative, glossy, substantially non-blocking and non-tacky, film, produced by the evaporation of the solvent from the lacquer composition defined in claim 2.

8. An article comprising a base at least one of the surfaces of which is coated with a protective and decorative, glossy, substantially non-blocking and non-tacky, film, produced by the evaporation of the solvent from the lacquer composition defined in claim 3.

9. An article comprising a base at least one of the surfaces of which is coated with a protective and decorative, glossy, substantially non-blocking and non-tacky, film, produced by the evaporation of the solvent from the lacquer composition defined in claim 4.

10. An article comprising a base at least one of the surfaces of which is coated with a protective and decorative, glossy, substantially non-blocking and non-tacky, film, produced by the evaporation of the solvent from the lacquer composition defined in claim 5.

11. A protective and decorative composition of the lacquer type as defined in claim 1 which includes a plasticizer.

12. A protective and decorative composition of the lacquer type as defined in claim 2 which includes a plasticizer.

13. A protective and decorative composition of the lacquer type as defined in claim 3 which includes a plasticizer.

14. A protective and decorative composition of the lacquer type as defined in claim 4 which includes a plasticizer.

15. A protective and decorative composition of the lacquer type as defined in claim 5 which includes a plasticizer.

16. A protective and decorative composition of the lacquer type defined in claim 1 and in which the alkali metal aliphatic sulphate is sodium lauryl sulphate.

17. A protective and decorative composition of the lacquer type defined in claim 2 and in which the alkali metal aliphatic sulphate is sodium lauryl sulphate.

18. A protective and decorative composition of the lacquer type defined in claim 3 and in which the alkali metal aliphatic sulphate is sodium lauryl sulphate.

19. A protective and decorative composition of the lacquer type defined in claim 4 and in which the alkali metal aliphatic sulphate is sodium lauryl sulphate.

20. A protective and decorative composition of the lacquer type defined in claim 5 and in which the alkali metal aliphatic sulphate is sodium lauryl sulphate.

CLEVELAND B. HOLLABAUGH.